

## UNITED STATES PATENT OFFICE

2,114,151

## ART OF FINISHING FERROUS METAL

Gerald C. Romig, Elkins Park, Pa., assignor to  
American Chemical Paint Company, Ambler,  
Pa., a corporation of Delaware

No Drawing. Continuation of application Serial  
No. 748,839, September 13, 1934. This applica-  
tion July 9, 1935, Serial No. 30,469

18 Claims. (Cl. 148—6.5)

This invention relates to the art of finishing ferrous metal and its principal object is to provide a final finish the life of which is materially lengthened due to greatly increased resistance to the destructive effects of corrosion or mechanical strain.

A further object of the invention is to provide a ferrous metal surface with a coating of paint, varnish, lacquer, Japan or the like, the life of which coating is greatly increased and its adhesion promoted, especially, as stated, where it may be subjected to atmospheric corrosion or mechanical strain.

An additional object is to produce finishes of very high luster with very thin coatings of paint or the like.

Still another object is the provision of a process for the finishing of metallic surfaces which will avoid the formation of hard, adherent incrustations on the vat, heating coils or other equipment used in treating the metal especially where this equipment is made of steel or other corrodible metal.

Another object is to increase the longevity of the protection afforded by temporary finishes such as oil, grease, wax, water-paint, white-wash, etc.

In connection with all of the foregoing objects it is a further important object of my invention to remove oil and grease from the surface of the metal while simultaneously providing it with a paint preservative coating.

Attention is called to the fact that this application is a continuation of my earlier application Serial No. 748,839, filed September 13, 1934.

I have discovered that chromic acid in solution may be activated so as to produce the desirable effect of increasing the longevity of finishes applied to ferrous metal surfaces.

Broadly speaking, the invention consists in treating the metallic surfaces to be finished with a solution containing chromic acid and one or more of a number of activating substances to be specified hereinbelow by dipping, brushing, spraying, mopping, etc., drying it with or without washing but preferably with washing in order to free the surface of the water soluble residues of the treating operation, and then coating it with paint, varnish, lacquer, Japan or other like material. In connection with the process the treated surface, before it is painted, may acquire a coating which may range from a transparent yellow discoloration to a heavy yellow to brown matte or layer, although in some cases the surface undergoes no change apparent to the eye. The

resulting color will depend on the temperature and time of treatment as well as upon the composition and concentration of the solution.

Generally stated the activating substance is an anion which acts catalytically to increase the action of the chromic acid solution on the metal. In my search for activator anions I have found that chloride, bromide, iodide, fluoride and ferricyanide anions are highly effective. Ferricyanide ions are immediately oxidized to ferricyanide and thus become equivalents of the latter. Broadly, therefore, my treating solution comprises chromic acid and one or more of the foregoing activating ions.

It should be noted, however, that the presence in the solution of moderate amounts of inorganic anions such as sulphate, phosphate, borate, etc., or of cations such as those of the alkali and alkaline earth metals, iron, zinc, cadmium, copper, mercury, etc., is not detrimental, although none of these ions is essential to the operation of the process, nor do any of them act as activator ions. The essential ingredients of my improved treating process are chromic acid and anions of the "activator type" above described by which are meant halogen ions, ferricyanides, and others which produce my desired result.

I have found in general that the desired effect can be obtained from solutions which contain at least .03 gram equivalents of activator anions per liter. Furthermore, the most generally applicable solution also contains free chromic acid, although in certain instances the presence of dichromates of certain metals such as zinc, iron, etc., furnishes sufficient acidity to operate the process and in such cases only the minimum quantity of activator anions need be present. However, solutions in which no free chromic acid is present are primarily useful only in instances where the surface to be treated is thoroughly degreased.

In the more generally applicable solutions, which contain free chromic acid, the concentration of activator anions should be at least two-tenths the concentration of the free chromic acid by weight. Four times as much activator anion as of free chromic acid or more may be used, but excessive amounts of activator anions lead to a decrease in the effectiveness of the treatment and I prefer to use activator anions at a concentration of from two-tenths to four times those of the free chromic acid, provided that a minimum of .03 gram equivalents of activator anion per liter is present.

5

10

15

20

25

25

30

35

35

40

40

45

45

50

50

55

55

Chromic acid behaves as a monobasic acid toward Brom-Cresol Green indicator, the dichromates of the alkalies being barely alkaline and zinc dichromate barely acid toward this indicator. 5 For the purpose of the present disclosure, therefore, I consider the "free" chromic acid in the solution to be that quantity of the chromic acid present which is capable of being titrated with caustic soda solution before the development of 10 a green color when using Brom Cresol Green as the indicator. "Combined" chromic acid is considered to constitute all of the chromic acid present "not free" as defined above.

As a specific example, I will describe my improved process as it may be applied to the coating of a steel stamping, such as an automobile fender.

The stamping as it comes from the press is generally contaminated with mill oil, grease, and/or drawing compound, and these impurities 20 may be removed by any of the well known conventional cleaning processes if so desired, but the process of my invention makes it possible to eliminate such a precleaning step. If precleaning is resorted to, scale and rust may be removed 25 with an acid pickle followed by washing with water, and oil and grease may be removed by wiping or washing with an oil solvent or by boiling in a bath of an alkaline cleaner.

However, if the stamping does not bear objectionably heavy rust or scale, it is unnecessary to resort to such a precleaning step as stated above, provided that the treatment hereinafter described is thoroughly effected. My treatment will remove oil and grease and even though scale or 35 rust are not removed, I have discovered that it will produce very satisfactory paint life without the necessity of any precleaning step. In the case of scale or rust the treatment apparently removes or renders harmless the corrosion stimulative materials and while tightly adherent scale or rust may interfere somewhat with the smoothness of the final finish, it will not stimulate further corrosion.

Furthermore, it should be noted that my improved process is quite insensitive to any precleaning method which may be used because the desired effect may be obtained equally well on pickled metal, on alkali-cleaned metal, or on metal cleaned by washing or wiping with solvent, or 50 on metal which has not been precleaned.

A solution is prepared in accordance with the following formula in connection with which, as well as in connection with all of the formulas given hereinbelow, the quantity of chromic acid specified is given in terms of the anhydride, CrO<sub>3</sub>, since chromic acid, H<sub>2</sub>CrO<sub>4</sub>, is not a stable, weighable compound:

Formula No. 1

|                                     |      |       |
|-------------------------------------|------|-------|
| 60 Chromic acid (CrO <sub>3</sub> ) | lb.  | 0.033 |
| Common salt                         | lb.  | 0.167 |
| Water, to make                      | gal. | 1.000 |

Sufficient of the solution of the foregoing formula is prepared to fill the tank of one section of a conventional metal-washing machine, and preferably heated to a temperature between about 120° and 200° F. and preferably in the neighborhood of 180° F., although the solution may be employed at any temperature up to its boiling point, to which end the tank is provided with some suitable means of heating, such, for example, as steam coils.

I prefer to wash the treated surface before applying the final finish because I find that to

do so improves the character of the finish. To this end, therefore, a second section of the washing machine is filled with water which may be cold or may be heated to accelerate the drying of the washed stampings. The stampings are then passed through the washing machine by a conveyor or other suitable means, the pumps of the washing machine being operated to keep jets of the solution and the water impinging strongly on the stampings in the respective sections. 10

The stampings should be subjected to the impinging action of the solution in the first stage of the washing machine for approximately 1 minute or thereabouts although the time required for the completion of the treating operation may vary somewhat with the temperature, the concentration of the solution and the nature of the metal being treated, etc., but none of these factors is critical as long as the chromic acid and the activator ion are present in the proper concentration. It might also be stated that an increase in the time of treatment apparently is without effect when the treatment has been properly performed in accordance with this disclosure. 20

The treatment is of distinct advantage over prior practices familiar to the art especially where equipment of a corrodible nature is employed, such as a steel vat with heating coils, because with my improved process no serious incrustation of the vat, heating coils or other equipment occurs. This is a distinct advantage over processes employing solutions of phosphates in which a heavy stone-like incrustation soon covers the vat and the heating coils or other equipment, 30 which incrustation, of course, interferes greatly with the transmission of heat through the solution and necessitates frequent draining and cleaning of the vat. It should be noted, however, that in the case of steel equipment, the solution 40 has a tendency to cause a certain degree of corrosion although this is not so serious as to preclude its use in metallic apparatus of this kind. However, such corrosion entails a useless consumption of chemicals and where metallic vats and coils are employed, it is preferable to construct them of some non-corrodible material such as stainless steel. 45

After the treatment in the washing machine the stampings are dried. This may be accomplished by any convenient means, but it is preferable to dry the stampings at an elevated temperature, as for instance, in an oven which may be maintained at any temperature below that which will cause oxidation of the steel with the consequent formation of a scale. When dry the stampings are ready for the application of a final coating of paint, lacquer, varnish, japan, or the like, in accordance with any of the practices familiar to the art. 50

In some instances a coating produced by the above solution will be sufficiently thick to interfere with the smoothness or luster of the applied finish coats and if this be so a weaker solution 55 may be employed having, for instance, half the concentration of the solution of Formula No. 1 as given above.

The solution of Formula No. 1 in the process just described is quite vigorous in its action and in order to reduce the violence of this action as well as to "buffer" the solution and to furnish an auxiliary supply of potentially "free" chromic acid I prefer to add to the solution, in addition to the free chromic acid and activator anion, 70

chromic acid combined with a metal or metals capable of forming water insoluble normal or basic chromates.

Such solutions will then contain chromate ions, activator anions, sufficient hydrogen ion to be capable of titration as "free" chromic acid, in accordance with the above definition, and ions of a metal or metals which are capable of forming insoluble basic or normal chromates.

Among the metals whose dichromates have been used to successfully buffer these solutions are zinc, cadmium, calcium, aluminum, iron, chromium, manganese and copper. Solutions prepared in this way have the further advantage that they produce the desired effect on the longevity and adhesion of applied finishes with less attack on the metal undergoing treatment and this results in economy of chemicals consumed and reduces the frequency of testing and of additions of reagents.

A solution, buffered as described, is given below:

*Formula No. 2*

|                                  |      |       |
|----------------------------------|------|-------|
| Chromic acid (CrO <sub>3</sub> ) | lb.  | 0.042 |
| Zinc dichromate                  | lb.  | 0.202 |
| Sodium chloride                  | lb.  | 0.083 |
| Water, to make                   | gal. | 1.000 |

This solution is ready for use, although for economy in shipping and storage it may be prepared in concentrated form by mixing the chromic acid with about .15 gallon of water and stirring in zinc oxide and sodium chloride gradually, in the proper proportions, until dissolved, after which the concentrated solution may be diluted to conform to the above formula before it is used.

Another useful formula is given below:

*Formula No. 3*

|                 |      |        |
|-----------------|------|--------|
| Chromic acid    | lb.  | 0.0500 |
| Ferric chloride | lb.  | 0.0700 |
| Common salt     | lb.  | 0.0750 |
| Water, to make  | gal. | 1.0000 |

As mentioned above, certain types of metal surface may be processed in solutions containing no "free" chromic acid. In these solutions the chromic acid can be considered to be present as the dichromates of one or more metals. Activator anions must be present in a concentration of at least 0.03 gram equivalents per liter, although concentrations as high as 0.10 gram equivalents or more are permissible. However, the results obtained are less satisfactory when the concentration of activator anion exceeds 0.07 gram equivalents per liter. These solutions produce practically effective results only when the metals are entirely free of grease or other contaminants when treated. A solution containing no free chromic acid which is suitable for treating grease-free steel, may be made as follows:

*Formula No. 4*

|                 |      |        |
|-----------------|------|--------|
| Chromic acid    | lb.  | 0.2500 |
| Zinc oxide      | lb.  | 0.1067 |
| Sodium chloride | lb.  | 0.0333 |
| Water, to make  | gal. | 1.0000 |

The process, using this formula, is similar to that described in the previous examples. It is essential, however, when using this solution, to subject the metal to be treated to a very thorough cleaning, as for instance, by suspending it for a short time in a vapor degreaser. Under favorable conditions, the results produced by this solution are excellent.

The process of this invention using any of the

foregoing formulas, produces, on the metal, a visible chromate coating of a yellowish to brownish color.

All the illustrative formulas given above, as well as others within the scope of this disclosure, may be prepared by dissolving appropriate amounts of dry admixtures in the correct amounts of water. For instance, the solution of Formula No. 1 may be prepared as follows:

*Formula No. 5*

|                                  |     |       |
|----------------------------------|-----|-------|
| Chromic acid (CrO <sub>3</sub> ) | lb. | 0.333 |
| Common salt                      | lb. | 0.667 |

The above dry admixture may be conveniently and economically shipped in sealed containers. When it is to be used it is dissolved in enough water to yield four gallons of a solution identical with that of Formula No. 1.

Another method of preparing a dry admixture is to evaporate to dryness a concentrated solution such as that given under Formula No. 2. The resulting residue, reduced to particles of convenient size, serves, on solution in the appropriate amount of water, to reproduce the solution of Formula No. 2.

The solutions of any of the above formulas may be applied by any method which will cause them properly to wet the surfaces to be treated. However, where no precleaning step is employed more or less vigorous mechanical treatment may be found necessary to achieve thorough wetting of the surface of the metal, and this, of course, will depend somewhat upon the nature and quantity of the contaminating materials which are present. For instance, the treating solution may be applied by flowing, brushing, mopping, or wiping of the surface with or submerging it in the solution as well as by impingement of jets of the solution in a washing machine as described above. In case such procedures are adopted, certain obvious precautions may become necessary. As the speed of any chemical process is largely affected by the temperature, it will be necessary to increase the time of treatment as the effective temperature of the surface is lowered. This is exemplified by the directions under Formula No. 2. It is sometimes useful when the treatment of the surfaces is carried out in the cold to use solutions more concentrated than those given in the examples. Such changes, however, will be obvious to one skilled in the art.

In addition to its value in producing long-lived finishes generally, my process has the advantage of making possible the production of finishes of very high luster with very thin coatings of paint, varnish, lacquer, japan or the like. Moreover, incidental scratches or other injuries to the finished surfaces are prevented from spreading under the organic coating material. Furthermore, as stated above, the treating process of this invention is useful in increasing the longevity of the protection afforded by temporary finishes such as oil, grease, wax, water, paint, whitewash, etc. which are often applied during fabrication or while awaiting the application of the final finish.

I claim:

1. The method of finishing the surface of ferrous metal which comprises forming a chromate coating thereon by treating it with a solution containing chromic acid and activator anions from the class which consists of halogens and ferricyanides, and applying to the coated surface a finish of paint, varnish, lacquer, japan, or the like.

2. The method of finishing the surface of ferrous metal which comprises forming a chromate coating thereon by treating it with a solution containing free chromic acid and activator anions from the class which consists of halogens and ferricyanides, and applying to the coated surface a finish of paint, varnish, lacquer, japan, or the like.
3. The method of finishing the surface of ferrous metal which comprises forming a chromate coating thereon by treating it with a solution containing free chromic acid and activator anions from the class which consists of halogens and ferricyanides, the concentration of the activator anions in the solution being from about two-tenths to four times the concentration of the free chromic acid, by weight, but not less than .03 gram equivalents per liter, and applying to the coated surface a finish of paint, varnish, lacquer, japan, or the like.
4. The method of claim 2 wherein the solution also contains dichromate of at least one metal of the class which consists of zinc, cadmium, calcium, aluminum, iron, chromium, manganese, and copper.
5. The method of claim 3 wherein the solution also contains dichromate of at least one metal of the class which consists of zinc, cadmium, calcium, aluminum, iron, chromium, manganese, and copper.
6. The method of finishing the surface of ferrous metal which comprises forming a chromate coating thereon by treating it with a solution containing free chromic acid and sodium chloride, the concentration of the chloride ion from the sodium chloride, being from about two-tenths to four times the concentration of the free chromic acid, by weight, but not less than .03 gram-equivalents per liter, washing and drying the coated surface, and then applying a finish of paint, varnish, lacquer, japan, or the like.
7. The method of finishing the surface of ferrous metal which comprises forming a chromate coating thereon by treating it with a solution containing free chromic acid, zinc dichromate and sodium chloride, the concentration of the chloride ion from the sodium chloride, being from about two-tenths to four times the concentration of the free chromic acid, by weight, but not less than .03 gram-equivalents per liter, washing and drying the coated surface, and then applying a finish of paint, varnish, lacquer, japan, or the like.
8. The method of finishing the surface of iron or steel which comprises forming a chromate coating thereon by treating it with a solution of approximately the following composition:
- Chromic acid ( $\text{CrO}_3$ ) ..... lb. 0.083  
Common salt ..... lb. 0.167  
Water, to make ..... gal. 1.000
- washing and drying the coated surface and then applying a finish of paint, varnish, lacquer, japan, or the like.
9. The method of finishing the surface of iron

or steel which comprises forming a chromate coating thereon by treating it with a solution of approximately the following composition:

|                                 |      |       |   |
|---------------------------------|------|-------|---|
| Chromic acid ( $\text{CrO}_3$ ) | lb.  | 0.042 | 5 |
| Zinc dichromate                 | lb.  | 0.202 |   |
| Sodium chloride                 | lb.  | 0.083 |   |
| Water, to make                  | gal. | 1.000 |   |

washing and drying the coated surface, and then applying a finish of paint, varnish, lacquer, japan, or the like.

10. The method of finishing the surface of iron or steel which comprises forming a chromate coating thereon by treating it with a solution of approximately the following composition:

|                                 |      |        |    |
|---------------------------------|------|--------|----|
| Chromic acid ( $\text{CrO}_3$ ) | lb.  | 0.2500 | 15 |
| Zinc oxide                      | lb.  | 0.1067 |    |
| Sodium chloride                 | lb.  | 0.0333 |    |
| Water, to make                  | gal. | 1.0000 | 20 |

washing and drying the coated surface and then applying a finish of paint, varnish, lacquer, japan, or the like.

11. A ferrous metal article having on a surface thereof a finish of paint or the like applied to an integral coating of the composition resulting from the treatment of claim 1.

12. A ferrous metal article having on a surface thereof a finish of paint or the like applied to an integral coating of the composition resulting from the treatment of claim 2.

13. A ferrous metal article having on a surface thereof a finish of paint or the like applied to an integral chromate coating having the composition resulting from treating the article with a solution containing free chromic acid and activator anions from the class which consists of halogens and ferricyanides wherein the concentration of activator anions in the solution is between about two-tenths and four times the concentration of the free chromic acid, by weight, but not less than .03 gram-equivalents per liter of the treating solution.

14. A ferrous metal article having on the surface thereof a finish of paint or the like applied to an integral coating of the composition resulting from the treatment of claim 6.

15. A ferrous metal article having on the surface thereof a finish of paint or the like applied to an integral coating of the composition resulting from the treatment of claim 7.

16. A ferrous metal article having on a surface thereof a finish of paint or the like applied to an integral coating of the composition resulting from the treatment of claim 8.

17. A ferrous metal article having on a surface thereof a finish of paint or the like applied to an integral coating of the composition resulting from the treatment of claim 9.

18. A ferrous metal article having on a surface thereof a finish of paint or the like applied to an integral coating of the composition resulting from the treatment of claim 10.